

Jan. 11, 1938.

R. LATTORF

2,105,152

ARTIFICIAL SLAB

Filed Sept. 4, 1935



Inventor

Richard Lattorf

by

Potter, Pierce & Scheffler  
his attorneys

## UNITED STATES PATENT OFFICE

2,105,152

## ARTIFICIAL SLAB

Richard Lattorf, Hanover, Germany, assignor  
to The United Limmer and Vorwohle Rock  
Asphalte Company Limited, London, England,  
a British company

Application September 4, 1935, Serial No. 39,189  
In Germany April 13, 1934

## 2 Claims. (Cl. 94—15)

This invention relates to artificial stone slabs, such as are used for the paving of floors or other building purposes both inside and out of doors.

Known forms of slabs, composed of hydraulic mortar, are often defective in that floors and pavings made thereof are very cold for the feet. In addition such floors are very good sound conductors, and when walked upon tend to reverberate the sound of the footsteps to a considerable extent.

The object of the invention is to provide an artificial stone slab which shall have a high insulating capacity against transmission of heat and sound, and which may be rapidly and cheaply produced.

According to this invention there is provided an artificial stone slab, the upper or wearing surface of which is formed of granular natural stone with a matrix of hydraulic mortar, preferably of Portland cement mortar, united with an underlayer consisting of asphalt or of a mass containing asphalt. An artificial stone slab in accordance with the invention is illustrated in the accompanying drawing.

The invention moreover includes an artificial stone slab characterized in that the artificial stone mass contains filling materials of granular rough texture, in order to ensure complete penetration into the asphalt mass and a good key therefor.

In this specification the term "asphalt" includes natural asphalt, or synthetic asphalt, or asphalt mastics.

In one embodiment of the invention the unification of the artificial stone mass and the asphalt underlayer is effected in a single operation under high compression of about seven thousand to eight and a half thousand pounds per square inch; the artificial stone mass is preferably applied with a minimum content of water, that is to say with a humidity approximating to that of soil.

The following description, given by way of example, shows one way in which these slabs may be made.

In moulds, which are preferably situated on a rotating table, and which are open at the top, there is first of all spread a layer of asphalt powder, suitably heated, to a thickness of about three-quarters to one inch. If desired other ingredients may be mixed with the asphalt powder. The artificial stone is then spread on this layer to any desired thickness, preferably about three-quarters of an inch to an inch and a half. The matrix of the said artificial stone is composed of

hydraulic mortar, and preferably of Portland cement; if desired a high quality rapid hardening cement, e. g. the so-called rapid super hard cement, may be used. The filling material consists of an aggregate of a granular rough material such as natural stone chippings with a rough sharp surface. The artificial stone mass (consisting of a mixture of about one part cement and from one to three parts stone aggregate) is preferably used in a stiff doughy condition, i. e. with a minimum water content. It is therefore in a condition approximating to that of moist earth. Immediately upon the application and spreading of this artificial stone mass a high compression is exerted upon both layers. This compression amounts to about seven thousand to eight and a half thousand pounds per square inch.

Under the action of this high compression, the two layers are intimately combined and penetrate into one another at the point of contact. In a way the layers grow into one another inasmuch as the two masses which are still plastic intimately combine during the application of the compression; and, since they penetrate into one another to a certain extent, there is no regular line of demarcation between the stone and the asphalt when a slab is seen in cross-section, but the line is of a broken character because at various points the respective layers have a greater or lesser penetration, thus affording an excellent key with each other. The excellence of this key is obviously to be ascribed to the use of the granular rough filling material in the artificial stone mass, and also to the plasticity and yielding quality of the compressed asphalt mass. This method of manufacture produces a very durable composite slab and renders possible mass production on an economical and rapid basis.

Although the underlayer is preferably composed of asphalt powder, it is also possible to manufacture the underlayer from mastic asphalt by casting, or from suitable masses having a considerable asphalt content. The stone aggregate may suitably be composed of any natural mineral stone which has a granular rough texture.

The foregoing description relates only to slabs in which compression is used to unite the two layers; an alternative method, without using high compression other than mere manual pressure or tamping, is to apply the artificial stone mass in a more liquid form to an underlayer composed mainly of cast mastic asphalt, with or without suitable filling materials embodied in it for purposes of insulation; this method of construction

has the advantage of being cheap and simple, and does not involve the use of expensive machinery.

The said filling material may consist of cork, 5 asbestos, pumice, wood, peat and similar fibrous materials, and is intended to form an insulation against heat, cold and reverberation.

The following description, given by way of example, shows one method of making the slabs 10 according to the above embodiment.

The hot asphalt is poured into moulds to a thickness of about three-quarters of an inch to one inch. Small pieces of insulating materials of the kind above-mentioned are fixed in the 15 asphalt before it is poured out. While it is in the moulds, and is still hot and comparatively liquid, dry grit is sprinkled upon it and combines therewith inseparably. This is done to provide a rough and unequal surface to afford a key for 20 the artificial stone layer which is subsequently to be applied in a fairly liquid consistency.

After the cast asphalt has been cooled (either by air or by water), the artificial stone mortar mass is applied in a liquid consistency approximating to that of plaster, to a depth of about three quarters of an inch to an inch and a half.

The gritty and roughened surface of the cast asphalt underlayer gives an excellent key with the cement mortar mass, and when the latter 30 has set it becomes inseparable from the underlayer. The surface of the artificial stone mass is smoothed off level with the top of the moulds before it has finally set hard.

Slabs constructed as above described afford excellent insulation both against extremes of temperature, moisture and reverberation. Owing to the elasticity of the asphalt underlayer increased 35 breaking resistance is also obtained.

The surface of the artificial stone slab may obviously be finished in various ways; it may, for example, be tessellated, and may have various designs and/or colouring incorporated, and also a separate coating layer.

The lower face of the asphalt underlayer may be smooth, roughened or shaped in any desired manner.

The slabs themselves are laid in mortar in the 10 normal manner.

What I claim and desire to secure by Letters Patent is:—

1. An artificial stone unit for building purposes comprising a layer of substantial thickness consisting of granular natural stone with a matrix 15 of hydraulic mortar and a layer of substantial thickness of a mass containing asphalt, characterized in that the slab consists solely of the two layers united directly together so that the one layer is keyed or bonded into the other, the first-mentioned layer forming the wearing surface of the slab, while the asphalt-containing layer forms the base of the slab for attachment directly to the surface on which the slab is laid, at least a 20 part of the particles of granular natural stone having a rough texture and being of sufficient size to key the two layers together.

2. Tile covering, characterized by the fact that it is composed of a two-layer unit, the wearing layer of which is of substantial thickness and is 30 formed of granular natural stone with a matrix of hydraulic mortar united directly with an underlayer of substantial thickness consisting of a mass containing asphalt, at least a part of the 35 particles of granular natural stone having a rough texture and being of sufficient size to key the two layers together.

RICHARD LATTORF.